# EUROPEAN PATENT SPECIFICATION

(11) **EP 0 862 990 B1**
(45) Date of publication and mention of the grant of the patent: **10.09.2003**
(21) Application number: 97830086.1
(22) Date of filing: 28.02.1997
(51) Int. Cl.: B32B 1/00, B27N 3/28, B27N 3/00

(54) **Apparatus for the continuous production of wood-based laminates**
Vorrichtung zur kontinuierlichen Herstellung von auf Holz basierenden Laminaten
Dispositif pour fabriquer en continu des laminates à base de bois

(43) Date of publication of application: 09.09.1998
(73) Proprietor: Valenti, Impero, 47100 Forli' Fo (IT)
(72) Inventor: Valenti, Impero, 47100 Forli' Fo (IT)
(74) Representative: Lanzoni, Luciano

(56) References cited:
- EP-A- 0 426 619
- GB-A- 388 387
- GB-A- 586 198
- GB-A- 880 198
- US-A- 4 112 145
- US-A- 5 096 046
- PATENT ABSTRACTS OF JAPAN vol. 009, no. 168 (M-396), 13 July 1985 & JP 60 042009 A (SADAO NISHIBORI), 6 March 1985,

## Description

The present invention relates to an apparatus for the continuous production, starting from a malleable agglomerate, of wood-based laminates for veneering and wainscoting.

As is well known, wooden furniture is, in the vast majority of cases, wainscoted with thin wooden laminates, obtained by shearing directly off the wood used. These laminates are utilised to manufacture furniture and also as wainscoting materials. The work process for these laminates is quite complex and naturally, given the nature of wood, it entails a large quantity of scrap.

Document US-A-4 112 145 discloses a method for manufacturing a lining material capable of replacing materials such as wood veneering wherein a malleable mixture mainly comprising wood powder and a vinyl glue and obtained by accurately mixing the various components, is forcibly inserted under rolling cylinders, a press, or the like, to turn the mixture into a uniform, thin layer. The layer may be subsequently embossed or ingraved to give it a particular appearance (such as that of wood grain) and cut into sheets of the desired length. The composition of the malleable mixture may further comprise diluents or solvents, various inert mineral charges, a lubricating oil, and other additives, such as coloring, flame-proof or anti-electrostatic products.

Document EP-A-0 426 619 discloses an apparatus for manufacturing remoldable, self- supporting, thin wood based panels comprising kneading sections for integral mixing of a thermoplastic polymer and wood flour and extruding stations for multiply extruding the mixture in a thin laminated wood panel. The extruded thin wood panel thus obtained is further fed into a conventional calender and then passed to a cutter.

Document GB-A-388 387 depicts an apparatus comprising a kneading section, an extrusion section and a laminating station.

The purpose of the invention is to eliminate the drawbacks stated above, providing a wood-base laminate, less expensive and with the elimination of scrap.

The present invention is an agglomerate constituted essentially by extremely fine wooden particles (wood flour), of an average diameter of about 75 micron and inert components closely linked to each other by aceto-vinyl resins.

The high wood content, as well as the particular production technique, allow to obtain a material that is truly alternative to natural wood.

The subject laminate can be produced in thicknesses ranging from 0.3 mm and 0.5 mm, depending on the envisioned use.

During the productive phase, the surface of the laminate undergoes an engraving or embossing process, in order to imitate more realistically the grain of the chosen wood; without such embossing, it can be lacquered directly.

The laminate has characteristics which are wholly similar to a normal wood in regard to gluing and painting, with the advantage of an enormously lower porosity.

It is easily heat-moulded starting at the temperature of 20/30°C, and this can be exploited advantageously to wainscot curved surfaces, frames, etcetera; with the aid of a hot air source, the laminate can be modelled and adapted for gluing on any kind of support.

Since the laminate can be heat-moulded, it can be provided for use in the form of rolls, but also in the form of sheets cut to the required size. The subject laminate, though it is made up to a large extent of wood, is very advantageously fire-proof and thus not flammable.

The laminate is also water-proof, it cannot be attacked by mildews and it can be stored in a cool, dry place for an indefinite time without being subject to phenomena of dimensional, colour, or other kind of alteration.

The laminate is also sound-absorbing, and therefore well suited for masonry walls and public places.

The laminate can be glued to various supports with the use of slow adhesives with pressure drying or with rapid adhesives like Bostic; it can be polished with polyurethane- or polyester-based polishes.

It can be used for furniture, supported on faesite, plywood, multi-layers and sheet metal; it can be used on suitably prepared masonry walls, it is very well suited to cover frames with any kind of curve or corner, for wainscoting any plane and knickknacks; it remains unchanged over time, i.e. it is not subject to the shrinking, cracking and swelling which are characteristic of normal wood.

The cost-effectiveness of the laminate with respect to normal veneering stems from the lower cost of the material (though only an expert would be able to recognise the difference), from the possibility of having it in the required size and thickness, without the wastage associated with true veneering; from the lessened a need to prepare the surface for painting.

These results are obtained thanks in part to a special apparatus, which allows a high continuous hourly production of the subject laminate.

By means of the subject apparatus, it is possible automatically to prepare the starting malleable agglomerate which, once it has transited through a laminating station to obtain the required thickness, is treated to disperse volatile components either in a natural or forced way, recovering the said components for the initial recycling.

Lastly, in addition to the possible stations engraving the laminate with the desired wood grain, cutting station is also provided to finish the laminates in the desired sizes. These laminates can be collected both in the form of sheets, and of reeled rolls. In both cases, the laminates are protected by appropriate protective plastic sheaths.

Additional characteristics and advantages of the invention shall be made clearer in the detailed description which follows, illustrated purely by way of non limiting example in the enclosed drawings, in which:
- Figure 1 and 1.1 are a schematic rendition of the entire subject apparatus;
- Figure 2 shows an alternative cutting station of the subject apparatus;
- Figure 3 shows a schematic detail of the starting set for the preparation of the agglomerate, as per Figure 1;
- Figure 4 shows a schematic detail of the calendering station as per Figure 1;
- Figure 5 shows a schematic detail of the engraving station as per the apparatus in Figure 1;
- Table 1 shows the composition of the starting agglomerate in the two variants of non fire-proof and fire-proof agglomerate, with the related minimum and maximum percentages;
- Tables 2 and 2A show five sample embodiments of the starting agglomerate, of which the first three examples refer to the fire-proof agglomerate and the last two examples refer to the non fire-proof agglomerate.

With reference to the enclosed drawings and tables, the apparatus for the continuous production of the subject laminate essentially comprises, in succession, a starting set 1 for preparing the malleable agglomerate, a laminating station 2, fed by the set 1 and able to transform the agglomerate into a thin layer 23 and a cutting station 6, able to reduce the thin layer 23 into laminates 68 of the required size.

It is appropriate first of all to define the components of the said malleable agglomerate.

It is composed, essentially, in the manner reported in Table 1. In practice its main component is a very fine wood powder, which can thus be defined as wood flour, with average granule size of about 75 micron and in a percentage ranging from 23% to 30%.

With the wood flour it is necessary to mix an adhesive of thermoplastic material, in order to provide a certain thermoplasticity to the finished product as well; the adhesive is present in a percentage ranging from 10% to 12%.

The adhesive used is vinyl resin, and in particular the adhesive designated "K115" by MONTEDISON or "MOWILITH 90" by HOECHST.

In the agglomerate are also present inert mineral charges, to render the laminate more compact and stronger, in a percentage ranging from 5% to 13%.

The agglomerate requires a lubricating agent, of the paraffin-based type, in a percentage ranging from 1 to 1.6%.

Lastly, diluting agents are necessary, which will volatilise in the course of agglomerate manufacturing, in a percentage ranging from 48% to 58%.

Should it be necessary to produce, as is clearly preferable, a fire-retarding and thus non flammable agglomerate, the components are the same as above, with the appropriate addition of fire-retarding materials, which will thus move the percentages in the way also indicated in Table 1.

Given that the agglomerate according to the present invention must be such as not to adhere to any support during the process whereby the laminate is formed with the subject apparatus, the presence of said lubricant contributes to this goal, such lubricant being specifically zinc stearate, but a contribution is also provided by the inert mineral charge of talc, always present in the agglomerate. In any case, the inert materials of the agglomerate may also be chosen among calcium carbonate (example 4), or silica-, carbonate-, magnesium- and manganese-based compounds, all materials present in the powder derived from diatoms, a particular type of shells (example 2). This latter component is particularly interesting, since in the agglomerate it is rather spongy and thus easily absorbs liquids for a successful agglomerate but also lets the liquids and the diluting agents easily volatilise during the drying and laminating process which will be described further on. More in particular, aluminium hydroxide can be found in the product known as "APYRAL" BY VAW AG BOON - (GERMANY); ammonium polyphosphate can be identified with the product "exolit 422" by GREAT LAKES INDIANA - (U.S.A.); diatom powder can be found in the product "CELITE 281" by JOHN MANVILLE (U.S.A.).

The fire-proof materials pertaining to non-flammable agglomerates in particular, are chosen among bromine-based compounds, such as decabromodiphenyloxide, commercially available for instance as "DER 83" by GREAT LAKES INDIANA (example 2); antimony-based compounds, such as antimony sesquioxide (example 1); phosphorus salts-based compounds, such as ammonium polyphosphate which, as mentioned above, is also an inert charge (example 2); chlorine-based compounds, such as chloroparaffin or chlorinated paraffin, available commercially as "cloroparaffina 70" manufactured by the Italian firm CAFFARO (example 1); aluminium-based compounds such as aluminium hydroxide or APYRAL (example 1). This last compound is useful above all because it reduces the emission of fumes, without developing aggressive or toxic products, and its endothermic decomposition develops a large quantity of water, diluting atmospheric oxygen, without adding to unburned byproducts and carbon residues.

With regard to the aforesaid lubricant, i.e. zinc stearate, it should be remembered that this product is a thermoplastic material and therefore contributes to the final plasticity of the laminate. With regard to the diluting agents, they comprise trichloroethane and turpentine in proportions which may vary approximately from 8:1 to 15:1. While trichloroethane essentially serves as a pure diluting agent, turpentine in practice acts as a solvent. In the course of the laminate formation process, these diluting agents will be eliminated from the final product by means of volatilisation and recovered to be reused in the cycle.

The examples of embodiment reported in Tables 2 and 2A entail precise percentages of products which fall within the scope of the possibilities of forming an agglomerate which is suitable for the purpose. Percentage variations according to the invention are choices made depending on the application of the final laminate, depending on the greater or lesser plasticity to be obtained and thus on how easily it is to be heat-moulded, depending on the hardness of the material to be obtained and, of course, depending on whether it is to be flammable or non-flammable. Naturally, the fire-retarding material requires more components, but it is by far preferable to the non fire-proof material. Having described the malleable agglomerate to be worked on, we shall return to the apparatus for its manufacture. The starting set 1 also uses a set 9 for triturating the wood, which is then entered into a fine grinding set 10 to obtain the said wood flour.

The starting set 1 comprises a first station 11 for the calibrated distribution of the compounds of the agglomerate which are in the solid and/or powdery state, such as the wood flour, the vinyl resin related to the adhesive, the inert materials, etcetera, while a second calibrated distribution station 12 is destined to the compounds of the agglomerate which are in the liquid state, such as the diluting agents and, for instance, the "DER 83".

Downstream of the calibrated distribution station 11 and 12 are respective mixers 13 and 14, for mixing the compounds coming, in the exact quantity required, from the said distribution stations. Lastly, there is a kneading machine 15, which receives the various materials and is able to form the malleable agglomerate automatically and to feed it to the subsequent lamination station 2.

In particular, each calibrated distribution station is fitted, for each compound, with a containment silos 16, associated to its own device 17 for weighing the compound, in order to feed it to the corresponding mixer 13 or 14, in the pre-set, exact quantity, independently from the other compounds, through a distribution way 18 or 18'.

The mixers 13 and 14 and each weighing device 17 are commanded electrically by a microprocessor circuit 19, in order always to provide the correct doses to the kneading machine 15, regardless of the quantity required. The kneading machine 15, which is actuated by a gearmotor 151, performs its function of mixing all compounds by means of a rotating fork 152. Next to the kneading machine 15 is a stand-by tank 20 connected to it, able to store and feed material to the lamination distribution 2, replacing the kneading machine 15 during the latter's down time.

The material formed by the kneading machine 15 or coming from the stand-by tank 20 is transferred to the subsequent laminating station 2 by means of a screw conveyer 151 and 201.

The lamination station 2 instead comprises, in succession, an extruder 21, which forms an agglomerate layer formed along the horizontal direction, and a calendering station 22, able to determine the definitive thickness of the layer which will constitute the final laminate.

The calendering station 22 comprises at least a pair of motor-driven roller sets 221, 222, facing each other and oriented downward. One of them and preferably the one next to the extruder 21 (see Figure 4), is fixed, while the other one (222) is movable with respect to the first. In particular it has to create a through-passage section 211 in the agglomerate layer exiting from extruder 21, in order to reduce it to a thin thickness 23, which is the definitive one of the laminate to be obtained. Of course, the through-passage section shall be adjustable and, for example, the movable roller set can be pivoting, around a hinge 225 coinciding for instance with the axis of the roller at the larger height. The roller sets are preferably fully encompassed by continuous belts 223 and 224, which of course are movable along the direction of flow of the agglomerate layer. The two roller sets shall be moved by chains 226, motor-driven along the direction of rotation of the arrows F1 and F2.

Downstream of the calendering station 222 is a conveyor belt 227 placed at the output side of the roller sets and able to transfer the thin agglomerate layer towards the subsequent stations.

The layer exiting the calendering station 22 could, in theory, be transferred directly to the cutting station 6, if the agglomerate layer were to be dried naturally or if waiting periods were possible. However, since this apparatus must be designed for a large hourly production, it is evident that, between the calendering station 22 and the cutting station, it is necessary to have additional stations able to accelerate the drying process of the agglomerate layer. Moreover it is always possible to produce engravings on the laminate to imitate the classic grain of the wood being worked or of another type of wood and therefore it is best to include a station 4 for engraving the agglomerate layer exiting the calendering station 22. It restores on the layer the typical grain of the wood used in the work process or it produces other grains and it is preceded, in the example depicted, by a forced ventilation station 3, which comprises at least a fan 31 and a hood 32 placed over it to collect volatilisation products and to render the agglomerate layer suitable to be permanently engraved.

The subsequent engraving station 4 comprises (see Figure 5) at least a first fixed roller 41 and a second rotating and engraved counter-roller 42, whose position with respect to the first roller can be adjusted according to the thickness of the agglomerate layer to be engraved, which passes between the two rollers. The adjustable roller is connected for instance with a handwheel 42 which, actuating for instance worm screws 44 which engage the support 45 of the engraved rotating counter-roller, causes it to move away from or towards the fixed roller 41.

Downstream of the engraving station 4, there is a rapid drying station 5, to disperse in a short time all the volatile products which were used to constitute an effective initial agglomerate. It comprises a ventilated chamber 51, in which one or more fans 53 send forced air inside the chamber 51, and at least one exit 54 for the volatile products, which, as shall be made clear further on, are all conveyed inside a single collection hood 7, from which the volatile products are collected by a recovery device 8, so they can be re-entered into the cycle, through the starting set 1.

Inside the ventilated chamber 51 there is a number of conveyor belts 52 stacked one above the other, along which, in a limited horizontal space, the horizontal layer can develop along a back and forth path for a large extension, in order to expose its surface for a long time to the action of the forced air circulation, which carries away with it all volatile products to be dispersed.

At the output of the drying station 5, through one or more conveyor belts T, the cutting station 6 is reached, which comprises a slitting machine 61 to determine the lateral cuts of the finished laminate, and a vertical shear 62 able instead to determine the transverse cuts of the laminate 68.

In order to protect the laminates thus produced, there is a reel 63 feeding a plastic sheath 69, also subject to the cuts made by the vertical shear 62. Downstream of the cutting station 6 is a counter 64 for packaging the laminate, cut in overlaid sheets, vertically movable in height, in order to support a pile of laminates, each with its own plastic sheath interposed. Since the laminate is a thermoplastic product, it can advantageously be collected in reels 66. In this case, the packaging counter 65 comprises at least one reel 66 for the collection of the laminate and of the protection sheath 69 and it also comprises at least an additional stand-by reel 67.

Moreover, since the process for laminating the subject agglomerate must unfold without any snags, the agglomerate must necessarily be insofar as possible free of adherence to the various supports it encounters during the process. This problem is for the most part solved by the paraffin-based lubricants present in the agglomerate itself and by the talc chosen as an inert mineral charge, but the apparatus itself is also provided with a design feature for this purpose. All conveyors T and the conveyors 52 of the rapid drying station 5 are made up of non-stick and fire-proof meshes. Lastly, it should be noted that the whole laminate forming process is advantageously carried out at ambient temperature, which should be no lower than 18/20°C.

Furthermore the whole apparatus, including the said microprocessor circuit 19 is run and regulated by a computerised electronic system (100), with synoptic display, which determines the adjustments of all the motor drives and/or regulation devices, such as the intervention time of the drying stations, the distances between the roller sets (221) and (222) etcetera. In practice, the computerised electronic system (100) runs and regulates the functional phases of the whole apparatus.

**TABLE 1**

| **AGGLOMERATE COMPOSITION NON FIRE-PROOF** | |
|---|---|
| **COMPOUND** | **MIN/MAX PERCENTAGES** |
| wood flour | 23% - 30% |
| adhesive | 10% - 12% |
| inert charges | 6% - 10% |
| lubricant | 1%- 1.6% |
| diluting agents | 48% - 58% |

| **FIRE-PROOF** | |
|---|---|
| **COMPOUND** | **MIN/MAX PERCENTAGES** |
| wood flour | 20% - 25% |
| adhesive | 7% - 12% |
| inert charges | 5% - 15% |
| lubricant | 1%- 1.6% |
| fire-retarding materials | 2.5% - 8% |
| diluting agents | 48% - 58% |

**TABLE 2**

| **EXAMPLES OF AGGLOMERATE COMPOSITION FIRE-PROOF** | |
|---|---|
| **EXAMPLE 1*** | |
| **COMPOUND** | **PERCENTAGES** |
| wood flour | 22.8% |
| vinyl resin | 8.9% |
| talc | 5.5% |
| aluminium hydroxide | 7.5% |
| antimony sesquioxide | 2% |
| chloroparaffin | 2% |
| zinc stearate | 1.5% |
| trichloroethane | 45.8% |
| turpentine | 4% |

| **EXAMPLE 2** | |
|---|---|
| **COMPOUND** | **PERCENTAGES** |
| wood flour | 23.8% |
| vinyl resin | 8.65% |
| talc | 4.9% |
| diatom powder | 1.1% |
| ammonium polyphosphate | 4.3% |
| decabromodiphenyloxide | 2.7% |
| zinc stearate | 1.6% |
| trichloroethane | 48.65% |
| turpentine | 4.3% |

| **EXAMPLE 3*** | |
|---|---|
| **COMPOUND** | **PERCENTAGES** |
| wood flour | 20.5% |
| vinyl resin | 11.2% |
| talc | 5.9% |
| decabromodiphenyloxide | 5.75% |
| antimony sesquioxide | 2% |
| zinc stearate | 1% |
| trichloroethane | 48.3% |
| turpentine | 5.35% |

| | |
|---|---|
| * not according to the invention | |

**TABLE 2A**

| **NON FIRE-PROOF** | |
|---|---|
| **EXAMPLE 4*** | |
| **COMPOUND** | **PERCENTAGES** |
| wood flour | 25.5% |
| vinyl resin | 11.2% |
| talc | 1% |
| calcium carbonate | 5.2% |
| zinc stearate | 1% |
| trichloroethane | 52.5% |
| turpentine | 3.6% |

| **EXAMPLE 5*** | |
|---|---|
| **COMPOUND** | **PERCENTAGES** |
| wood flour | 25% |
| vinyl resin | 11.5% |
| talc | 7% |
| zinc stearate | 1% |
| trichloroethane | 52% |
| turpentine | 3.5% |

| | |
|---|---|
| * not according to the invention | |

## Claims

1. Apparatus for the continuous production, starting from a malleable agglomerate, of wood-based laminates for veneering and wainscoting, comprising at least, in succession:
- a starting set (1) for the preparation of a malleable agglomerate composed of wood flours, adhesive and diluting agents:
- a laminating station (2), fed by the said set (1), able to transform the agglomerate into a thin layer (23);
- a cutting station (6), able to reduce the thin layer (23) into laminates (68) of the required size;
**characterised in that** the said starting set (1) comprises at least:
- a first station (11) for the calibrated distribution of the compounds of the agglomerate which are in the solid and/or powdery state;
- a second station (12) for the calibrated distribution of the compounds of the agglomerate which are in the liquid state;
- a first and a second mixer (13, 14), respectively able to provide prior mixing to the compounds coming, in the exact quantity required, from the said first arid second distribution station (11, 12);
- a kneading machine (15), able to form the malleable agglomerate and to feed it to the laminating station (2), mixing the material coming from the first calibrated distribution station (11) with the material which gradually arrives from the second calibrated distribution station (12) for the liquid compounds;
each calibrated distribution station (11, 12) being fitted, for each compound, with a containment silos (16), associated with a device (17) for weighing the compound, in order to feed the respective mixer (13, 14) with the pre-set and exact quantity of the specific compound, independently from the other compounds, by means of a corresponding distribution way (18) and (18').

2. Apparatus according to claim 1, **characterised in that** at least each mixer (13, 14) and each weighing device (17) are commanded electronically by a microprocessor circuit (19), so as always to provide the correct doses to the kneading machine (15), regardless of the quantity required.

3. Apparatus according to claim 1, **characterised in that** it is provided with a stand-by tank (20), connected to the kneading machine (15), able to store and to feed material to the laminating station (2) substituting for the kneading machine (15) and during its down-times.

4. Apparatus according to claim 1, **characterised in that** the laminating station (2) comprises at least in succession:
- an extruder (21) able to form a layer (211) of agglomerate developed along the horizontal direction;
- a calendering station (22), able to determine the definitive thickness of the layer.

5. Apparatus according to claim 4, **characterised in that** the calendering station (22) comprises a pair at least of motor-driven roller sets (221, 222) facing each other and oriented downward, at least one of which (222) is movable, in order to determine, with respect to the other, a through-passage section adjustable according to the required lamination thickness, at least one conveyor belt (223), located at the output side of the roller sets (221, 222) and provided to transfer the laminated agglomerate layer towards the subsequent stations.

6. Apparatus according to claim 5, **characterised in that** each roller set (221, 222) is encompassed by a continuous-loop belt (223, 224), movable according to the direction of flow of the agglomerate layer.

7. Apparatus according to claim 5 or 6, **characterised in that** the movable roller set (222) pivots, with a hinge (225) in its upper part, in order to determine, on its lower side, the required through-passage section.

8. Apparatus according to claims 1 or 4, **characterised in that** between the laminating station (2) and the cutting station (6) a station (4) is provided for engraving the agglomerate layer exiting the calendering station (22), able to restore, on the layer, the typical wood grain, said engraving station (4) being preceded by a forced ventilation station (3), able to render the agglomerate layer suitable to be permanently engraved by dispersing a part of its volatile components.

9. Apparatus according to claims 1 or 4 or 8, **characterised in that**, before the cutting station (6), a rapid drying station (5) is provided, able to disperse in a reduced amount of time all volatile products from the agglomerate layer.

10. Apparatus according to claim 8, **characterised in that** the engraving station (4) comprises at least a first fixed roller (41) and a second engraved rotating counter-roller (42), whose position with respect to the first can be adjusted according to the thickness of the agglomerate layer to be engraved.

11. Apparatus according to claim 9, **characterised in that** the drying station (5) comprises a ventilated chamber (51), within which a number of conveyor belts (52) are fitted, stacked one above the other, along which, in a horizontally limited space, the agglomerate layer can develop, along a back and forth path, for a large extension, in order to expose its surface for a long time to the action of the forced air circulation, which carries away with it the volatile products to be dispersed.

12. Apparatus according to claim 1, **characterised in that** the cutting station (6) comprises a slitting machine (61), able to determine the lateral cuts and a vertical shear (62) able to determine the transverse cuts of the agglomerate layer, thus defining the required size of the definitive laminate (68), and at least one reel (63) for feeding a plastic protection sheath (69), also subject to the cuts of the vertical shear (62).

13. Apparatus according to claim 12, **characterised in that** it comprises a counter (64) for packaging the laminate, cut in overlaid sheets, movable vertically in height.

14. Apparatus according to claim 12, **characterised in that** it comprises a counter (65) for packaging the laminate collected into reels, equipped with a reel (66) for collecting both the laminate and the protective sheath (69) and at least one stand-by reel (67).

15. Apparatus according to any one of the previous claims, **characterised in that** at least the transfer of the agglomerate from the starting set (1) to the laminating station (2) is accomplished by means of screw conveyers (151, 201), whereas in the subsequent stations it is accomplished by means of conveyor belts (T and 52) made up of non-stick, fire-retarding meshes.

16. Apparatus according to any one of the previous claims, **characterised in that** it comprises a single hood (7) for the collection of the diluting agents volatilised by the agglomerate when it is processed, and a device (8) to recover them, for their reinsertion in the cycle, through the starting set (1).

17. Apparatus according to claim 1, **characterised in that** the starting set (1) also employs a set (9) for triturating the wood, subsequently inserted in a fine grinding set (10), to obtain the wood flour.

18. Apparatus according to any of the previous claims, **characterised in that** it comprises at least one computerised electronic system (100), able to run and regulate all functional phases of production.

19. Malleable agglomerate for the production of wood-based laminates for veneering and wainscoating, comprising at least wood flour, adhesive of a thermoplastic material, inert mineral charges, paraffin-based lubricant, diluting agents, **characterised in that** wood flour is present in a percentage ranging from 23% to 30%, the adhesive of a thermoplastic material is present in a percentage ranging from 10% to 12%, inert mineral charges are present in a percentage ranging from 5% to 13%, paraffin-based lubricant is present in a percentage ranging from 1% to 1.6%, diluting agents are present in a percentage ranging from 48% to 58%, and **characterized in that** to the inert mineral charges is added a natural mineral charge obtainable from diatom powder and whose basic components are silica-based, carbonate-based, magnesium-based and manganese-based compounds.

20. Malleable agglomerate for the production of wood-based laminates for veneering and wainscoating, comprising at least wood flour, adhesive of a thermoplastic material, inert mineral charges, paraffin-based lubricant, fire-proof materials, diluting agents, **characterised in that** wood flour is present in a percentage ranging from 20% to 25%, the adhesive of a thermoplastic material is present in a percentage ranging from 7% to 12%, inert mineral charges are present in a percentage ranging from 5% to 15%, paraffin-based lubricant is present in a percentage ranging from 1% to 1.6%, fire-proof materials are present in a percentage ranging from 2.5% to 8%, diluting agents are present in a percentage ranging from 48% to 58%, and **characterized in that** to the inert mineral charges is added a natural mineral charge obtainable from diatom powder and whose basic components are silica-based, carbonate-based, magnesium-based and manganese-based compounds.

21. Agglomerate according to claim 19 or 20, **characterised in that** the adhesive is vynil resin.

22. Agglomerates according to claim 19 or 20, **characterised in that** the lubricant is a thermoplastic material made up of zinc stearate.

23. Agglomerate according to claim 19 or 20, **characterised in that** the diluting agents comprise at least trichloroethane and turpentine in proportions which may vary approximately from 8:1 to 15:1, respectively.

24. Agglomerate according to claim 19, **characterised in that** it is made up of at least the following components:
- wood flour;
- vinyl resin as an adhesive;
- talc as an inert mineral charge;
- zinc stearate as a lubricant;
- trichloroethane as a diluting agent and turpentine as a diluting agent - solvent.

25. Agglomerate as per claim 20, **characterised in that** fire-proof materials are chosen among: bromine-based compounds; antimony-based compounds; phosphorus salts-based compounds; chlorine-based compounds; aluminium-based compounds.

26. Agglomerate as per claim 20, **characterised in that** it includes at least the following specific components:
- wood flour,
- vinyl resin as an adhesive;
- talc and ammonium polyphosphate as an inert mineral charge;
- decabromodiphenyloxide and again ammonium polyphosphate, as fire-proof compounds;
- zinc stearate as a lubricant;
- trichloroethane as a diluting agent and turpentine as a diluting agent - solvent.

27. Agglomerate according to claim 20, **characterised in that** it includes at least the following specific components:
- wood flour,
- vinyl resin as an adhesive;
- talc as an inert mineral charge;
- decabromodiphenyloxide and antimony sesquioxide as fire-proof materials;
- zinc stearate as a lubricant;
- trichloroethane as a diluting agent and turpentine as a diluting agent - solvent.

28. Agglomerate according to claim 20, **characterised in that** it includes at least the following specific components:
- wood flour;
- vinyl resin as an adhesive;
- talc and aluminium hydroxide as inert mineral charges;
- again aluminium hydroxide, antimony sesquioxide and chloroparaffin as fire-proof materials;
- zinc stearate as a lubricant;
- trichloroethane as a diluting agent and turpentine as a diluting agent - solvent.

29. Agglomerate according to any one of the claims from 19 to 29, **characterised in that** the wood flours have a granule size of about 75 micron.

## Patentansprüche

1. Vorrichtung zur kontinuierlichen Herstellung, ausgehend von formbaren Agglomeraten, von auf Holz basierenden Laminaten für Furniere und Vertäfelungen, enthaltend aufeinanderfolgend wenigstens:
- eine Ausgangsvorrichtung (1) zum Zubereiten eines formbaren Agglomerats, bestehend aus Holzmehlen, Bindemitteln und Verdünnungsmitteln;
- eine Laminierstation (2), beschickt durch die genannte Vorrichtung (1) und in der Lage, das Agglomerat zu einer dünnen Schicht (23) zu verarbeiten;
- eine Schneidstation (6), in der Lage, die dünne Schicht (23) zu Laminaten (68) der gewünschten Abmessung zu reduzieren;
**dadurch gekennzeichnet, dass** die genannte Ausgangsvorrichtung (1) wenigstens wie folgt enthält:
- eine erste Station (11) zur dosierten Abgabe der Compounds des Agglomerats, die sich in einem festen und/oder pulverförmigen Zustand befinden;
- eine zweite Station (12) zur dosierten Abgabe der Compounds des Agglomerats, die sich in einem flüssigen Zustand befinden;
- einen ersten und einen zweiten Mischer (13, 14), jeweils vorgesehen zum Vormischen der Compounds in den genauen geforderten Mengen, die von der genannten ersten und der zweiten Abgabestation (11, 12) kommen;
- eine Knetmaschine (15), in der Lage, das formbare Agglomerat zu verarbeiten und an die Laminierstation (2) zu leiten, wobei sie das aus der ersten Station (11) zur dosierten Abgabe kommende Material mit dem Material mischt, das allmählich von der zweiten Station (12) zur dosierten Abgabe der flüssigen Compounds kommt;
wobei jede Station (11, 12) zur dosierten Abgabe für jedes Compound mit einem Vorratssilo (16) versehen ist, zugeordnet einer Vorrichtung (17) zum Abwiegen des Compounds, um den jeweiligen Mischer (13, 14) über einen entsprechenden Verteilerweg (18) und (18') mit der festgelegten und exakten Menge des spezifischen Compounds zu beliefern, und zwar unabhängig von den anderen Compounds.

2. Vorrichtung nach Patentanspruch 1, **dadurch gekennzeichnet, dass** wenigstens jeder Mischer (13, 14) und jede Wiegevorrichtung (17) elektronisch durch einen Mikroprozessorkreis (19) gesteuert werden, so dass unabhängig von der gewünschten Menge immer die korrekte Dosierung an die Knetmaschine (15) abgegeben wird.

3. Vorrichtung nach Patentanspruch 1, **dadurch gekennzeichnet, dass** sie mit einem Pufferbehälter (20) versehen ist, angeschlossen an die Knetmaschine (15) und in der Lage, Material zu speichern und an die Laminierstation (2) zu führen, und zwar als Ersatz für die Knetmaschine (15) und während den Stillstandphasen derselben.

4. Vorrichtung nach Patentanspruch 1, **dadurch gekennzeichnet, dass** die Laminierstation (2) aufeinanderfolgend wenigstens enthält:
- einen Extruder (21), in der Lage, eine Schicht (211) aus Agglomerat zu formen, die sich in einer horizontalen Richtung erstreckt;
- eine Kalanderstation (22), die dazu dient, die definitive Stärke der Schicht zu bestimmen.

5. Vorrichtung nach Patentanspruch 4, **dadurch gekennzeichnet, dass** die Kalanderstation (22) wenigstens ein Paar von angetriebenen Rollenbahnen (221, 222) enthält, die einander zugewandt und nach unten gerichtet sind, und von denen wenigstens eine beweglich ist, um im Verhältnis zu der anderen einen je nach der gewünschten Laminierstärke regulierbaren Durchlaufabschnitt zu bilden, sowie wenigstens ein Förderband (223), das am Ausgangsende der Rollenbahnen (221, 222) angeordnet und dazu vorgesehen ist, die laminierte Agglomeratschicht zu den anschliessenden Stationen zu transferieren.

6. Vorrichtung nach Patentanspruch 5, **dadurch gekennzeichnet, dass** jede Rollenbahn (221, 222) von einem ringförmig geschlossenen Band (223, 224) umgeben ist, beweglich in der Laufrichtung der Agglomeratschicht.

7. Vorrichtung nach Patentanspruch 5 oder 6, **dadurch gekennzeichnet, dass** die bewegliche Rollenbahn (222) an ihrem oberen Teil mit Hilfe eines Scharniers (225) angelenkt ist, um an ihrem unteren Teil den gewünschten Durchlaufabschnitt zu bestimmten.

8. Vorrichtung nach Patentanspruch 1 oder 4, **dadurch gekennzeichnet, dass** zwischen der Laminierstation (2 und der Schneidstation (6) eine Station (4) vorgesehen ist, um die aus der Kalanderstation (22) austretende Agglomeratschicht zu gravieren und somit auf der Schicht die typische Holzmaserung wiederherzustellen, wobei der genannten Gravierstation (4) eine Station (3) der forcierten Belüftung vorausgeht, um die Agglomeratschicht durch Dispersion eines Teils ihrer flüchtigen Komponenten geeignet für eine dauerhafte Gravierung zu machen.

9. Vorrichtung nach Patentanspruch 1 oder 4 oder 8, **dadurch gekennzeichnet, dass** vor der Schneidstation (6) eine Schnelltrockenstation (5) vorgesehen ist, in der Lage, innerhalb einer kurzen Zeit alle flüchtigen Produkte aus der Agglomeratschicht zu lösen.

10. Vorrichtung nach Patentanspruch 8, **dadurch gekennzeichnet, dass** die Gravierstation (4) wenigstens eine erste feststehende Walze (41) enthält sowie eine zweite gravierte, sich drehende Gegenwalze (42), deren Position im Verhältnis zu der ersten je nach der Stärke der zu gravierenden Agglomeratschicht reguliert werden kann.

11. Vorrichtung nach Patentanspruch 9, **dadurch gekennzeichnet, dass** die Trockenstation (5) eine belüftete Kammer (51) enthält, in welcher eine Anzahl von Förderbändern (52) vorgesehen ist, die eines über dem anderen liegen, und entlang welchen sich in einem horizontal begrenzten Raum die Agglomeratschicht auf Vor- und Rückwärtsbahnen über eine grosse Ausdehnung erstrecken kann, um ihre Oberfläche für eine lange Wirkungsdauer dem forcierten Luftumlauf auszusetzen, welcher die zu entfernenden flüchtigen Produkte mitnimmt.

12. Vorrichtung nach Patentanspruch 1, **dadurch gekennzeichnet, dass** die genannte Schneidstation (6) eine Schlitzmaschine (61) enthält, dazu bestimmt, die seitlichen Schnitte auszuführen, und eine vertikale Schermaschine, dazu bestimmt, die Querschnitte an der Agglomeratschicht auszuführen, wobei so die gewünschten Grössen des fertigen Laminates (68) hergestellt werden, sowie wenigstens eine Rolle (63) zum Zuführen einer Schutzfolie (69) aus Kunststoff, die ebenfalls den Schnitten der vertikalen Schermaschine (62) unterzogen wird.

13. Vorrichtung nach Patentanspruch 12, **dadurch gekennzeichnet, dass** sie einen Packtisch (64) zum Verpacken der zu übereinander liegenden Folien geschnittenen Laminate enthält, der vertikal in der Höhe beweglich ist.

14. Vorrichtung nach Patentanspruch 12, **dadurch gekennzeichnet, dass** sie einen Packtisch (65) zum Verpacken der zu Rollen gewickelten Laminate enthält, ausgestattet mit einer Wickelwalze (66) zur Aufnahme des Laminates und auch der Schutzfolie (69), sowie wenigstens eine Wickelwalze (67) als Reserve.

15. Vorrichtung nach einem beliebigen der vorstehenden Patentansprüche, **dadurch gekennzeichnet, dass** wenigstens der Transferieren des Agglomerats von der Ausgangsvorrichtung (1) an die Laminierstation (2) mit Hilfe von Schneckenförderern (151, 201) erfolgt, während es in den anschliessenden Stationen durch Förderbänder (T und 52) ausgeführt wird, hergestellt aus nicht haftenden und flammhemmenden Maschen.

16. Vorrichtung nach einem beliebigen der vorstehenden Patentansprüche, **dadurch gekennzeichnet, dass** sie eine einzige Haube (7) für den Abzug der Verdünnungsmittel enthält, die sich bei der Verarbeitung des Agglomerats verflüchtigt haben, und eine Vorrichtung (8) zur Wiedergewinnung derselben für ihre Wiedereingabe in den Zyklus durch die Ausgangsvorrichtung (1).

17. Vorrichtung nach Patentanspruch 1, **dadurch gekennzeichnet, dass** die Ausgangsvorrichtung (1) auch eine Vorrichtung (9) zum Vermahlen des Holzes verwendet, das anschliessend in eine Feinmahlvorrichtung (10) gegeben wird, um das Holzmehl zu erhalten.

18. Vorrichtung nach einem beliebigen der vorstehenden Patentansprüche, **dadurch gekennzeichnet, dass** sie wenigstens ein computerisiertes elektronisches System (100) enthält, in der Lage, alle Funktionsphasen der Produktion zu steuern und zu regulieren.

19. Formbares Agglomerat zur Herstellung von auf Holz basierenden Laminaten für Furniere und Vertäfelungen, enthaltend wenigstens Holzmehl, Bindemittel aus einem Kunststoffmaterial, träge Mineralfüllstoffe, auf Paraffin basierendes Gleitmittel und Verdünnungsmittel, **dadurch gekennzeichnet, dass** Holzmehl zu einem Anteil von 23% bis 30%, Bindemittel aus einem Kunststoffmaterial zu einem Anteil von 10% bis 12%, träge Mineralfüllstoffe zu einem Anteil von 5% bis 13%, auf Paraffin basierende Gleitmittel zu einem Anteil von 1% bis 1,6% und Verdünnungsmittel zu einem Anteil von 48% bis 58% vorhanden sind, und **dadurch gekennzeichnet, dass** den trägen Mineralfüllstoffen ein natürlicher Mineralfüllstoff zugefügt ist, erhältlich aus Diatomeenpulver, und dessen Basiskomponenten auf Silizium, Karbonat, Magnesium und Mangan basierende Compounds sind.

20. Formbares Agglomerat zur Herstellung von auf Holz basierenden Laminaten für Furniere und Vertäfelungen, enthaltend wenigstens Holzmehl, Bindemittel aus einem Kunststoffmaterial, träge Mineralfüllstoffe, auf Paraffin basierendes Gleitmittel, feuerfeste Materialien und Verdünnungsmittel, **dadurch gekennzeichnet, dass** Holzmehl zu einem Anteil von 20% bis 25%, Bindemittel aus einem Kunststoffmaterial zu einem Anteil von 7% bis 12%, träge Mineralfüllstoffe zu einem Anteil von 5% bis 15%, auf Paraffin basierende Gleitmittel zu einem Anteil von 1% bis 1,6%, feuerfeste Materialien zu einem Anteil von 2,5% bis 8% und Verdünnungsmittel zu einem Anteil von 48% bis 58% vorhanden sind, und **dadurch gekennzeichnet, dass** den trägen Mineralfüllstoffen ein natürlicher Mineralfüllstoff zugefügt ist, erhältlich aus Diatomeenpulver, und dessen Basiskomponenten auf Silizium, Karbonat, Magnesium und Mangan basierende Compounds sind.

21. Agglomerat nach Patentanspruch 19 oder 20, **dadurch gekennzeichnet, dass** das Bindemittel Vinylharz ist.

22. Agglomerat nach Patentanspruch 19 oder 20, **dadurch gekennzeichnet, dass** das Gleitmittel ein thermoplastisches Material, hergestellt aus Zinkstearat.

23. Agglomerat nach Patentanspruch 19 oder 20, **dadurch gekennzeichnet, dass** die Verdünnungsmittel wenigstens Trichlorethan und Terpentin in Verhältnissen enthalten, die jeweils zwischen 8:1 und 15:1 variieren können.

24. Agglomerat nach Patentanspruch 19, **dadurch gekennzeichnet, dass** es wenigstens aus den folgenden Komponenten besteht:
- Holzmehl;
- Vinylharz als Bindemittel;
- Talk als träger Mineralfüllstoff;
- Zinkstearat als Gleitmittel;
- Trichloethan als Verdünnungsmittel und Terpentin als Verdünnungs-/Lösungsmittel.

25. Agglomerat nach Patentanspruch 20, **dadurch gekennzeichnet, dass** die feuerfesten Materialien ausgewählt sind unter: Compounds auf der Basis von Brom, Antimon, Phosphorsalzen, Chlor und Aluminium.

26. Agglomerat nach Patentanspruch 20, **dadurch gekennzeichnet, dass** es wenigstens die folgenden spezifischen Komponenten enthält:
- Holzmehl;
- Vinylharz als Bindemittel;
- Talk und Ammonium-Polyphosphat als trägen Mineralfüllstoff;
- Dekabromdiphenyloxid und wieder Ammonium-Polyphosphat als feuerfeste Compounds;
- Zinkstearat als Gleitmittel;
- Trichlorethan als Verdünnungsmittel und Terpentin als Verdünnungs-/Lösungsmittel.

27. Agglomerat nach Patentanspruch 20, **dadurch gekennzeichnet, dass** es wenigstens die folgenden spezifischen Komponenten enthält:
- Holzmehl;
- Vinylharz als Bindemittel;
- Talk als trägen Mineralfüllstoff;
- Dekabromdiphenyloxid und Antimonsesquioxid als feuerfeste Materialien;
- Zinkstearat als Gleitmittel;
- Trichlorethan als Verdünnungsmittel und Terpentin als Verdünnungs-/Lösungsmittel.

28. Agglomerat nach Patentanspruch 20, **dadurch gekennzeichnet, dass** es wenigstens die folgenden spezifischen Komponenten enthält:
- Holzmehl;
- Vinylharz als Bindemittel;
- Talk und Aluminiumhydroxid als träge Mineralfüllstoffe;
- wieder Aluminiumhydroxid, Antimonsesquioxid und Chlorparaffin als feuerfeste Materialien;
- Zinkstearat als Gleitmittel;
- Trichlorethan als Verdünnungsmittel und Terpentin als Verdünnungs-/Lösungsmittel.

29. Agglomerat nach einem beliebigen der Patentansprüche von 19 bis 28, **dadurch gekennzeichnet, dass** das Holzmehl eine Körnung von etwa 75 µ hat.

## Revendications

1. Dispositif pour fabriquer en continu, à partir d'un agglomérat malléable, des laminates à base de bois pour le placage et le lambrissage, comprenant au moins, en succession:
- une installation initiale (1) pour la préparation d'un agglomérat malléable composé de farines de bois, adhésifs et diluants;
- une station de laminage (2), alimentée par ladite installation (1), pouvant transformer l'agglomérat en une fine couche (23);
- une station de coupe (6), pouvant réduire la fine couche (23) en laminates (68) de dimensions requises;
**caractérisé en ce que** ladite installation initiale (1) comprend au moins:
- une première station (11) pour la distribution calibrée des composés de l'agglomérat qui se présentent à l'état solide et/ou pulvérulent;
- une seconde station (12) pour la distribution calibrée des composés de l'agglomérat qui se présentent à l'état liquide;
- un premier et un second mélangeur (13, 14), chargés à mélanger préventivement respectivement les composants provenant, dans les exactes quantités requises, de la première et de la seconde stations de distribution (11, 12);
- une machine de malaxage (15), chargée de former l'agglomérat malléable et d'alimenter la station de laminage (2), en malaxant le matériau provenant de la première station calibrée de distribution (11) avec le matériau qui provient progressivement de la seconde station calibrée de distribution (12) pour les composés liquides;
chaque station calibrée de distribution (11, 12) étant équipée, pour chaque composé, d'un silo de contenance (16), associé à un dispositif (17) pour peser le composant, de manière à alimenter le mélangeur (13, 14) respectif avec une quantité exacte et prédéterminée du composé spécifique, indépendamment des autres composants, au moyen d'une correspondante voie de distribution (18) et (18').

2. Dispositif selon la revendication 1, **caractérisé en ce que** chaque mélangeur (13, 14) et chaque dispositif de pesage (17) sont commandés électroniquement par un circuit à microprocesseur (19), de manière à toujours fournir les doses correctes à la machine de malaxage (15), indépendamment de la quantité requise.

3. Dispositif selon la revendication 1, **caractérisé en ce qu'**il est pourvu d'un réservoir de réserve (20), relié à la machine de malaxage (15), pouvant stocker et alimenter en matériau la station de laminage (2) en substituant la machine de malaxage (15) et pendant ses arrêts.

4. Dispositif selon la revendication 1, **caractérisé en ce que** la station de laminage (2) comprend au moins en succession:
- une extrudeuse (21) pouvant former une couche (211) d'agglomérat développée en direction horizontale;
- une station de calandrage (22), pouvant déterminer l'épaisseur définitive de la couche.

5. Dispositif selon la revendication 4, **caractérisé en ce que** la station de calandrage (22) comprend au moins une paire de séries de rouleaux motorisés (221, 222) se faisant face et orientés vers le bas, au moins l'une desquelles (222) étant mobile, de manière à déterminer, par rapport à l'autre, une section de passage réglable selon l'épaisseur de laminage requise, au moins un tapis roulant (223), situé en sortie des séries de rouleaux (221, 222) et conçu pour transporter la couche d'agglomérat laminée vers les stations suivantes.

6. Dispositif selon la revendication 5, **caractérisé en ce que** chaque série de rouleaux (221, 222) est entourée d'une courroie continue en anneau (223, 224), mobile selon la direction du flux de la couche agglomérée.

7. Dispositif selon la revendication 5 ou 6, **caractérisé en ce que** la série de rouleaux mobiles (222) pivote, autour d'une charnière (225) dans sa partie supérieure, de manière à déterminer inférieurement la section de passage désirée.

8. Dispositif selon la revendication 1 ou 4, **caractérisé en ce que**, entre la station de laminage (2) et la station de coupe (6), est prévue une station (4) pour graver la couche agglomérée sortant de la station de calandrage (22), de manière à reproduire sur la couche le grain typique du bois, ladite station de gravure (4) étant précédée d'une station de ventilation forcée (3), servant à rendre la couche agglomérée adaptée à une gravure permanente en dispersant une partie de ses composants volatiles.

9. Dispositif selon la revendication 1, 4 ou 8, **caractérisé en ce que**, avant la station de coupe (6), est pourvue une station de séchage rapide (5) pouvant disperser en un temps réduit tous les produits volatiles de la couche agglomérée.

10. Dispositif selon la revendication 8, **caractérisé en ce que** la station de gravure (4) comprend au moins un premier rouleau fixe (41) et un second contre-rouleau rotatif gravé (42), dont la position par rapport au premier peut être réglée selon l'épaisseur de la couche agglomérée à graver.

11. Dispositif selon la revendication 9, **caractérisé en ce que** la station de séchage (5) comprend une chambre ventilée (51), dans laquelle est prévue une pluralité de tapis roulants (52), superposés, le long desquels, dans un espace horizontal limité, se développe la couche agglomérée, le long d'un parcours en avant et en arrière, sur une grande longueur, de manière à exposer sa surface pendant longtemps à l'action de la circulation d'air forcée, qui évacue les produits volatiles à disperser.

12. Dispositif selon la revendication 1, **caractérisé en ce que** la station de coupe (6) comprend une machine d'incision (61), servant à déterminer les coupes latérales, et une cisaille verticale (62) servant à déterminer les coupes transversales de la couche agglomérée, définissant ainsi la dimension requise du laminate définitif (68), et au moins une bobine (63) d'alimentation d'un voile plastique de protection (69), également objet de la coupe de la cisaille verticale (62).

13. Dispositif selon la revendication 12, **caractérisé en ce qu'**il comprend un banc (64) d'emballage du laminate, coupé en feuilles superposées, mobile verticalement.

14. Dispositif selon la revendication 12, **caractérisé en ce qu'**il comprend un banc (65) d'emballage du laminate recueilli en bobines, équipé d'une bobine (66) pour recueillir aussi bien le laminate que le voile protecteur (69) et d'au moins une bobine (67) de réserve.

15. Dispositif selon n'importe laquelle des revendications précédentes, **caractérisé en ce qu'**au moins le transfert de l'agglomérat de l'installation initiale (1) à la station de laminage (2) est accompli au moyen de convoyeurs à vis (151, 201), alors que dans les stations suivantes il est accompli au moyen de tapis roulants (T et 52) conformés en mailles anti-adhérentes et ignifuges.

16. Dispositif selon n'importe laquelle des revendications précédentes, **caractérisé en ce qu'**il comprend une unique hotte (7) pour la collecte des agents diluants volatilisés par l'aggloméré lorsqu'il est traité, et un dispositif (8) de récupération de ces derniers pour les réinsérer dans le cycle, au travers de l'installation initiale (1).

17. Dispositif selon la revendication 1, **caractérisé en ce que** l'installation initiale (1) emploie également une installation (9) de broyage du bois, ensuite inséré dans une installation de mouture fine (10) pour obtenir la farine de bois.

18. Dispositif selon n'importe laquelle des revendications précédentes, **caractérisé en ce qu'**il comprend au moins un système électronique informatisé (100), commandant et régulant toutes les phases fonctionnelles de production.

19. Agglomérat malléable pour la production de laminates à base de bois pour le placage et le lambrissage, comprenant au moins de la farine de bois, adhésif de matériau thermoplastique, charges minérales inertes, lubrifiant à base de paraffine, agents diluants, **caractérisé en ce que** la farine de bois est présente en un pourcentage de 23% à 30%, l'adhésif de matériau thermoplastique en un pourcentage de 10% à 12%, les charges minérales inertes en un pourcentage de 5% à 13%, le lubrifiant à base de paraffine en un pourcentage de 1% à 1,6%, les agents diluants en un pourcentage de 48% à 58%, et **caractérisé en ce qu'**est ajoutée aux charges minérales inertes une charge minérale naturelle obtenue de poudre diatomée et dont les composants basiques sont des composés à base de silice, carbonates, magnésium, manganèse.

20. Agglomérat malléable pour la production de laminates à base de bois pour le placage et le lambrissage, comprenant au moins de la farine de bois, adhésif de matériau thermoplastique, charges minérales inertes, lubrifiant à base de paraffine, matériaux ignifuges, agents diluants, **caractérisé en ce que** la farine de bois est présente en un pourcentage de 20% à 25%, l'adhésif de matériau thermoplastique en un pourcentage de 7% à 12%, les charges minérales inertes en un pourcentage de 5% à 15%, le lubrifiant à base de paraffine en un pourcentage de 1% à 1,6%, les matériaux ignifuges en un pourcentage de 2,5% à 8%, les agents diluants en un pourcentage de 48% à 58%, et **caractérisé en ce que** est ajoutée aux charges minérales inertes une charge minérale naturelle obtenue de poudre diatomée et dont les composants basiques sont des composés à base de silice, carbonates, magnésium, manganèse.

21. Agglomérat selon la revendication 19 ou 20, **caractérisé en ce que** l'adhésif est une résine vinyle.

22. Agglomérat selon la revendication 19 ou 20, **caractérisé en ce que** le lubrifiant est un matériau thermoplastique constitué de stéarate de zinc.

23. Agglomérat selon la revendication 19 ou 20, **caractérisé en ce que** les agents diluants comprennent au moins du trichloroéthane et de l'essence de térébenthine dans des proportions qui peuvent varier approximativement de 8:1 à 15:1, respectivement.

24. Agglomérat selon la revendication 19, **caractérisé en ce qu'**il est constitué d'au moins les composants suivants:
- farine de bois;
- adhésif sous forme de résine vinylique;
- charge minérale inerte sous forme de talc;
- lubrifiant sous forme de stéarate de zinc;
- diluant sous forme de trichloroéthane et diluant-solvant sous forme d'essence de térébenthine.

25. Agglomérat selon la revendication 20, **caractérisé en ce que** les matériaux ignifuges sont choisis parmi les matériaux suivants: composés à base de bromure, à base d'antimoine, à base de sels de phosphore, à base de chlore, à base d'alluminium.

26. Agglomérat selon la revendication 20, **caractérisé en ce qu'**il comprend au moins les composants spécifiques suivants:
- farine de bois;
- adhésif sous forme de résine vinylique;
- charge minérale inerte sous forme de talc et polyphosphate d'ammonium;
- composés ignifuges sous forme de décabromodiphényloxyde et encore polyphosphate d'ammonium;
- lubrifiant sous forme de stéarate de zinc;
- diluant sous forme de trichloroéthane et diluant-solvant sous forme d'essence de térébenthine.

27. Agglomérat selon la revendication 20, **caractérisé en ce qu'**il comprend au moins les composants spécifiques suivants:
- farine de bois;
- adhésif sous forme de résine vinylique;
- charge minérale inerte sous forme de talc;
- composés ignifuges sous forme de décabromodiphényloxyde et antimoine;
- lubrifiant sous forme de stéarate de zinc;
- diluant sous forme de trichloroéthane et diluant-solvant sous forme d'essence de térébenthine.

28. Agglomérat selon la revendication 20, **caractérisé en ce qu'**il comprend au moins les composants spécifiques suivants:
- farine de bois;
- adhésif sous forme de résine vinylique;
- charge minérale inerte sous forme de talc et d'hydroxyde d'aluminium;
- composés ignifuges sous forme encore d'hydroxyde d'aluminium, sesquioxyde d'antimoine et chloroparaffine;
- lubrifiant sous forme de stéarate de zinc;
- diluant sous forme de trichloroéthane et diluant-solvant sous forme d'essence de térébenthine.

29. Agglomérat selon n'importe laquelle des revendications 19 à 20, **caractérisé en ce que** les farines de bois sont sous forme de granulés d'environ 75 microns.
